

## UNITED STATES PATENT OFFICE

2,406,749

SIZING COMPOSITION AND YARN SIZED  
THEREWITH

Harry R. Dittmar, Wilmington, Del., assignor to  
E. I. du Pont de Nemours & Company, Wil-  
mington, Del., a corporation of Delaware

No Drawing. Application August 4, 1943,  
Serial No. 497,366

20 Claims. (Cl. 260—32)

**1**

This invention relates to a sizing composition and yarn sized therewith. More particularly, this invention relates to a sizing composition suitable for nylon yarns intended for the knitting of full-fashioned hosiery, and nylon yarn sized therewith.

It is known that the proper sizing of nylon yarn for use in the knitting of full-fashioned hosiery is a very critical operation. The basic requirements include (1) good knitting performance, even at high humidities, (2) good stitch formation, (3) no marked tendency of edge-rolling of the flat fabric since this makes seaming slow and expensive, and (4) excellent snag-resistance of the fabric throughout the several processing steps. One of the most successful of the sizing compositions available for nylon yarns is that described in U. S. patent of Edgar W. Spanagel, No. 2,324,601, issued July 20, 1943, and which consists of partially hydrolyzed polyvinyl acetate (known in the trade as polyvinyl alcohol) modified with a substantial but minor proportion of boric acid. Even this composition gives quite poor knitting performance under conditions of high humidity. This turns out to be a serious matter since high humidities prevail along the eastern seaboard for a considerable part of the year. Moreover, since it is good practice in knitting full-fashioned hosiery from silk to well humidify the yarn at the moment of knitting by passing it over a wick laden with water or through a chamber at 100% humidity, there is a strong tendency to do the same when working with nylon yarn. The result is that the ability to knit well at high humidities without depositing size on or fouling the knitting needles becomes the first criterion of a good knitting size.

It is an object of this invention to provide an improved sizing composition for nylon yarn to be used for the knitting of full-fashioned hosiery. Another object of this invention is to provide sized nylon yarn that will give good knitting performance even under conditions of high humidity. A specific object of this invention is to improve the polyvinyl alcohol-boric acid size so that nylon yarn sized therewith will knit well even at high humidities without depositing size on or fouling the needles or sinkers of the knitting machine. Other and additional objects will become apparent hereafter.

The objects of the invention are accomplished, in general, by modifying a polyvinyl alcohol-boric acid size by incorporating therein a modified polymer of dioxolane. The following examples are typical embodiments of the invention, and it is

**2**

to be understood that the invention is not restricted to the specific details thereof, the parts, proportions and percentages being by weight:

*Example I*

5 A size composition of the following ingredients in the proportions set forth is prepared in any convenient manner:

|                                 | Parts |
|---------------------------------|-------|
| 10 Polyvinyl alcohol-boric acid | 5     |
| Polydioxolane sebacate          | 5     |
| Water                           | 90    |

In the polydioxolane sebacate, the ratio of combined sebacic acid to combined 1,3-dioxolane is 1:8, and the compound has a molecular weight of about 1500 and a hydroxyl number of 61.7.

Single ends of 30 denier-10 filament-30 turn polyhexamethylene adipamide yarn is sized in conventional fashion with this composition to give a final yarn having 3.6% size and dried at 80° F. and 50% relative humidity for 9 hours. The yarn is twist-set in ovens at a dry bulb of 170° F. and a wet bulb of 165° F. for 2 hours, and thereafter conditioned at 72% relative humidity for 10 hours. It is finally coned, using a typical coning oil for nylon. It is knitted using a 45-gauge, single-end Wildman flat knitting machine, the yarn being conditioned at 100% relative humidity as knitting proceeds. The yarn runs very well through the knitting machine, leaving practically no deposit on the needles and latches even after several days' operation. The knitted stitches are well formed. The flat fabric remains substantially flat so that the seaming operation proceeds in a manner fully equal to the experience with natural silk. Overall mill performance shows a small percentage of pulled stitches due to snagging.

*Example II*

40 A composition of the following ingredients in the proportions set forth is prepared in any convenient manner:

|                                 | Parts |
|---------------------------------|-------|
| 45 Polyvinyl alcohol-boric acid | 6     |
| Polydioxolane adipate           | 4     |
| Water                           | 90    |

In the polydioxolane adipate, the ratio of combined adipic acid to combined 1,3-dioxolane is 1:10, and the compound has a molecular weight of about 1100 and a hydroxyl number of 66.7.

30 denier-10 filament-30 turn polyhexamethylene adipamide yarn is sized, dried, twist-set, conditioned, coned and knitted as set forth in Example I. During knitting, the running qualities of

this sized yarn are superior to nylon yarn sized with polyvinyl alcohol-boric acid size (without the modified dioxolane polymer) with no sacrifice in either the edge-rolling characteristics or the snag-resistance.

*Example III*

A composition of the following ingredients in the proportions set forth is prepared in any convenient manner:

|                              | Parts |
|------------------------------|-------|
| Polyvinyl alcohol-boric acid | 3.5   |
| Polydioxolane stearate       | 2.5   |
| Water                        | 94.0  |

In the polydioxolane stearate, the ratio of combined stearic acid to combined 1,3-dioxolane is 1:8, and the compound has a molecular weight of about 1200 and a hydroxyl number of 59.

Single ends of 30 denier-10 filament-30 turn polyhexamethylene adipamide are sized, dried, twist-set, conditioned and coned as set forth in Example I. The yarn is then knit as set forth in Example I except that the yarn is conditioned for knitting at a relative humidity of 50%, which is typical of certain parts of the year along the eastern seaboard. Completely satisfactory performance results.

The polyvinyl alcohol-boric acid of each of the above examples is a partially saponified polyvinyl acetate (known in the trade as polyvinyl alcohol) having a saponification number of 140 and a viscosity of 4 centipoises, modified with 20% boric acid based on the polyvinyl alcohol.

Though the examples refer to specific modified polymers of dioxolane, the invention is not restricted thereto. There may also be used polymers of dioxolane modified by other monobasic or polybasic carboxylic acids or esters thereof and prepared, for example, by (1) effecting the polymerization of the dioxolane in the presence of carboxylic acid, using a strong acid such as sulfuric acid for the catalyst; (2) first polymerizing the dioxolane in the presence of a strong acid such as sulfuric acid and then reacting it with an ester of the carboxylic acid, using an alkaline catalyst to obtain an alcoholysis reaction; and (3) first reacting dioxolane with the carboxylic acid to obtain a lower molecular weight polymer than desired and then subjecting this polymer to further reaction with dioxolane to obtain a higher molecular weight polymer. Similarly, substituted dioxolanes may be used as a starting material, and these include such compounds as the 2-ethyl and the 2,2-dimethyl 1,3-dioxolane. In general, the molecular weight of the modified dioxolane polymer should be within the range of 500 to 1500. The ratio of combined acid to the dioxolane may vary within quite wide limits. It will be obvious to one skilled in the art that if the ratio of the acid, such as stearic acid, becomes too large, the resulting polymer will not be soluble in water. Similarly, if the ratio of the acid is not properly chosen, the resulting polymer will not be a solid. The ratio within which water-solubility and a solid state is developed varies with the particular acid involved and is readily ascertainable by experiment. In every case, the dioxolane polymer intended for use with this invention should be a low-melting, waxy solid which is soluble in the water.

For a more detailed discussion of the method of preparation of these modified polymers of dioxolane, reference may be had to copending application Serial No. 395,366, filed May 27, 1941.

In the foregoing examples, preference has been

shown for a specific partially saponified vinyl acetate which is soluble or emulsifiable in water and which is known in the trade as polyvinyl alcohol. The invention, however, is not restricted to such specific polyvinyl alcohol. Generally speaking, any water-sensitive polyvinyl compound in which 1% to 50%, and preferably 35% to 50%, of the carbon atoms in the polyvinyl chain are attached to hydroxyl groups (such compounds being herein referred to as "hydroxylated polyvinyl resin") can be used. As illustrative examples of hydroxylated polyvinyl resins which can be used are the partial esters of polyvinyl alcohol such as the partial acetates, the partial propionates, the glycolic acid esters, the partial formates, and the partial lactates; the partial ethers of polyvinyl alcohol such as the glycol ethers, the glycolic acid ethers, the methyl ethers, and the ethyl ethers; the partial acetals of polyvinyl alcohol such as the partial formal, the partial acetal, the partial glyoxal, the partial propional, and the partial butyral; the partial ketals of polyvinyl alcohol such as the ethyl-methyl ketal.

Although partially saponified polyvinyl acetates having saponification numbers from 40 to 150 are particularly useful, partially saponified polyvinyl acetates having saponification numbers of between 10 and 300, such as 40 to 200, or even somewhat lower than 10 or higher than 300, may be used to advantage. Saponification numbers of the partially saponified polyvinyl acetate, as used herein, are defined as the number of milligrams of potassium hydroxide required to completely saponify 1 gram of the sample.

The partially saponified polyvinyl acetate may have viscosities of 1.5 to 20 centipoises, and preferably 4 to 6 centipoises, the viscosity being determined on a 4% aqueous solution at 20° C. using a Hoepppler viscosimeter.

In general, the amount of boric acid can vary within wide limits. The maximum quantity of boric depends on the characteristics of the particular hydroxylated polyvinyl resin and is sufficient to insure good running properties but insufficient to cause gelation. Although particularly desirable results are obtained when the boric acid constitutes approximately 20% to 22.5% of the weight of the polyvinyl alcohol, the amount of boric acid can vary between 5% and 25% based on the weight of the polyvinyl alcohol, the limit depending on the characteristics of the particular polyvinyl alcohol and being, on the one hand, sufficient to insure good running properties and, on the other hand, insufficient to cause gelation. When formals of polyvinyl alcohol containing 10% to 30% of formal constitute the hydroxylated polyvinyl alcohol, the amount of boric acid may vary from 5% to 20% based on the weight of the formal.

The proportions of the polyvinyl hydroxylated resin-boric acid composition to the dioxolane polymer may be varied within limits. In most cases, proportions of 50:50 seem to give optimum results, but quite satisfactory results are secured within the limits of 65:35 and 35:65.

It is true that the polyvinyl alcohol-boric acid composition by itself is quite a remarkable size for nylon yarn in terms of edge-rolling prevention and snag-resistance but its running characteristics at high humidities, as has been previously noted, are not at all satisfactory. The dioxolane polymers by themselves have no special sizing value and have extremely poor snag-resistance. It is quite surprising that they can so

materially improve the running qualities of the polyvinyl alcohol-boric acid composition without impairing the edge-rolling characteristics and the snag-resistance.

It will be obvious to one skilled in the art that the sizing compositions of this invention can be applied by conventional methods from an aqueous solution or dispersion of any desirable concentration to yield on the yarn a coating of any reasonable thickness. Solutions of 2% to 12% total solids content are preferred, depending, as is known, on such factors as the denier and filament count of the yarn, its water-sensitivity, the rate of travel of the yarn through the sizing bath, the temperature of the bath and of the drying conditions and the amount of size desired on the yarn. It will be obvious too that the amount of size desired on the yarn will vary with these or similar factors. Generally, a coating on the yarn of from 1% to 6% is preferred.

For reasons of simplicity, the invention has been discussed specifically in terms of polyhexamethylene adipamide yarn since that is the common nylon yarn of the market. The invention obviously embraces other synthetic linear polyamide yarns as well as related synthetic linear polymer yarns, such, for example, as those derived from polymerizable mono amino carboxylic acids or their amide-forming derivatives and those derived from the reaction of suitable diamines with suitable dicarboxylic acids or amide-forming derivatives of dibasic carboxylic acids, disclosed in U. S. Patents Nos. 2,071,250, 2,130,523 and 2,130,948. Without limiting the broad and general definitions of nylon as used elsewhere in patents or literature, the synthetic linear polyamides herein disclosed are defined as set forth in U. S. Patent 2,359,877, i. e. a synthetic linear polycarbonamide wherein the average number of carbons in the segments of the chain separating the amide groups is at least two.

The invention is additionally applicable to any water-insensitive synthetic linear polymer yarn, since the compositions employed in this invention adhere well to these yarns in contrast to the more well-known compositions. By the term "water-insensitive," it is meant that the individual filaments of the yarn absorb less than 10% of their weight of water at 25° C. and 100% relative humidity. Examples of such polymers are the vinyl chloride-vinyl acetate interpolymers, polymerized methyl methacrylate or polymerized ethyl methacrylate, polyvinyl chloride, chlorinated polyvinyl chloride, high molecular weight ethylene polymers, vinyl chloride-vinylidene chloride copolymers, and acrylonitrile and copolymers thereof.

The invention has special value in connection with the knitting of full-fashioned hosiery since that involves very fine and delicate yarns, careful knitting, the problem of edge-rolling of the flat fabric with the difficulty of seaming, and the chances of snagged and pulled threads inherent in the many processing steps. The composition of the invention is basically an excellent knitting size for water-insensitive yarns, as discussed, and equally useful for circular knitting of similar or heavy fabrics from similar or heavy denier yarns, including monofil, and also may be used to advantage with other structures, such as films, staple fiber, spun yarn, mixed yarn, ribbons, etc.

By reason of the invention, the expeditious knitting of nylon yarns into such critical fabrics as full-fashioned hosiery is more fully assured. Orderly and more regular knitting is maintained.

Even when knitting at high relative humidities, as is commonly done, or when knitting at uncontrolled humidities which sometimes show great variations from day to day or even from hour to hour in some parts of the eastern seaboard, the composition of this invention assures regular and excellent knitting with no fouling of the knitting needles or sinkers and no perceptible wear on the needles, even after several days of operation. It is difficult to define the excellence of the knitting performance in mathematical language, but it can be stated that the sizing composition of this invention gives as good knitting performance at 100% humidity as the best previous compositions gave with dry knitting.

The subsequent process steps can be easily carried out and the percentage of damaged stockings materially decreased. The invention involves no new equipment or altered techniques. The control of the edge-rolling of the flat fabric is also entirely satisfactory, as can be seen from a seaming time for 100 stockings of 80 minutes, compared with 98 minutes with the best previous composition knit dry as against the knitting according to this invention at 100% humidity. The protection of the fabric against snagging and pulled threads during the subsequent processing steps is quite satisfactory, taking into consideration the excellent knitting performance. Based on 1,000 stockings carried through knitting, seaming, boil-off, boarding and drying, the compositions of this invention show 10% to 14% pulled threads as against 0% to 20% for the best previous sizing composition, i. e. polyvinyl alcohol-boric acid. It might be interesting to note in passing that when these modified polymers of dioxolane are used by themselves, the percentage of pulled threads was 61%, an intolerable situation.

As a matter of fact, the resistance of workers to working on nylon stockings in view of their inherent difficulties compared with silk has been finally overcome. Significant to the public is the fact that the cost of stockings bears a close relationship to the percentage of stockings made that cannot leave the factory because of pulled threads or snagging in the processing. One of the attributes of this invention is that this percentage is materially decreased.

Since it is obvious that many changes and modifications can be made in the above-described details without departing from the nature and spirit of the invention, it is to be understood that the invention is not to be limited thereto except as set forth in the appended claims.

55 I claim:

1. A yarn-sizing composition comprising a water-sensitive hydroxylated polyvinyl resin, boric acid and a polymer of the class which consists of modified polymers of dioxolane and alkyl substituted dioxolanes, said polymer being a water-soluble waxy solid having a molecular weight within the range of 500 to 1500 and modified by a member of the class which consists of carboxylic acids and esters thereof, the ratio of the total amount of said hydroxylated resin and boric acid to the amount of said polymer being within the limits of 65:35 and 35:65.

2. A yarn-sizing composition comprising an aqueous solution of a water-sensitive hydroxylated polyvinyl resin, boric acid and a polymer of the class which consists of modified polymers of dioxolane and alkyl substituted dioxolanes, said polymer being a water-soluble waxy solid having a molecular weight within the range of 500 to 1500 and modified by a member of the class

which consists of carboxylic acids and esters thereof, the ratio of the total amount of said hydroxylated polyvinyl resin and boric acid to the amount of said polymer being within the limits of 65:35 and 35:65, and the boric acid being present in an amount of from 5% to 25% based on the weight of the hydroxylated polyvinyl resin.

3. A yarn-sizing composition comprising a partially saponified polyvinyl acetate, boric acid and a polymer of the class which consists of modified polymers of dioxolane and alkyl substituted dioxolanes, said polymer being a water-soluble waxy solid and having a molecular weight within the range of 500 to 1500 and modified by a member of the class which consists of carboxylic acids and esters thereof, the ratio of the total amount of said polyvinyl acetate and boric acid to the amount of said polymer being within the limits of 65:35 and 35:65.

4. A yarn-sizing composition comprising a partially saponified polyvinyl acetate, boric acid and a polymer of the class which consists of modified polymers of dioxolane and alkyl substituted dioxolanes, said polymer being a water-soluble waxy solid having a molecular weight within the range of 500 to 1500 and modified by a member of the class which consists of carboxylic acids and esters thereof, the ratio of the total amount of said polyvinyl acetate and boric acid to the amount of said polymer being within the limits of 65:35 and 35:65, and the boric acid being present in an amount of from 5% to 25% based on the weight of the polyvinyl acetate.

5. A yarn-sizing composition comprising a partially saponified polyvinyl acetate, boric acid and polydioxolane sebacate, the ratio of the total amount of said polyvinyl acetate and boric acid to the amount of said polydioxolane sebacate being within the limits of 65:35 and 35:65.

6. A yarn-sizing composition comprising a partially saponified polyvinyl acetate, boric acid and polydioxolane sebacate, said polydioxolane sebacate having a molecular weight of about 1500, a hydroxyl number of 61.7 and a ratio of combined sebacic acid to combined 1,3-dioxolane of 1:8, the ratio of the total amount of said polyvinyl acetate and boric acid to the amount of said polydioxolane sebacate being within the limits of 65:35 and 35:65.

7. A yarn-sizing composition comprising a partially saponified polyvinyl acetate, boric acid and polydioxolane adipate, the ratio of the total amount of said polyvinyl acetate and boric acid to the amount of said polydioxolane adipate being within the limits of 65:35 and 35:65.

8. A yarn-sizing composition comprising a partially saponified polyvinyl acetate, boric acid and polydioxolane adipate, said polydioxolane adipate having a molecular weight of about 1100, a hydroxyl number of 66.7 and a ratio of combined adipic acid to combined 1,3-dioxolane of 1:10, the ratio of the total amount of said polyvinyl acetate and boric acid to the amount of said polydioxolane adipate being within the limits of 65:35 and 35:65.

9. A yarn-sizing composition comprising a partially saponified polyvinyl acetate, boric acid and polydioxolane stearate, the ratio of the total amount of said polyvinyl acetate and boric acid to the amount of said polydioxolane stearate being within the limits of 65:35 and 35:65.

10. A yarn-sizing composition comprising a partially saponified polyvinyl acetate, boric acid and polydioxolane stearate, said polydioxolane stearate having a molecular weight of about 1200, a

hydroxyl number of 59 and a ratio of combined stearic acid to combined 1,3-dioxolane of 1:8, the ratio of the total amount of said polyvinyl acetate and boric acid to the amount of said polydioxolane stearate being within the limits of 65:35 and 35:65.

11. A water-insensitive yarn having a size coating comprising a water-sensitive hydroxylated polyvinyl resin, boric acid and a polymer of the class which consists of modified polymers of dioxolane and alkyl substituted dioxolanes, said polymer being a water-soluble waxy solid, having a molecular weight within the range of 500 to 1500, and modified by a member of the class which consists of carboxylic acids and esters thereof, the ratio of the total amount of said hydroxylated resin and boric acid to the amount of said polymer being within the limits of 65:35 and 35:65.

12. A water-insensitive yarn having a size coating comprising a water-sensitive hydroxylated polyvinyl resin, boric acid and a polymer of the class which consists of modified polymers of dioxolane and alkyl substituted dioxolanes, said polymer being a water-soluble waxy solid, having a molecular weight within the range of 500 to 1500, and modified by a member of the class which consists of carboxylic acids and esters thereof, the ratio of the total amount of said hydroxylated polyvinyl resin and boric acid to the amount of said polymer being within the limits of 65:35 and 35:65.

13. A water-insensitive yarn having a size coating comprising a partially saponified polyvinyl acetate, boric acid and a polymer of the class which consists of modified polymers of dioxolane and alkyl substituted dioxolanes, said polymer being a water-soluble waxy solid, having a molecular weight within the range of 500 to 1500, and modified by a member of the class which consists of carboxylic acids and esters thereof, the ratio of the total amount of said polyvinyl acetate and boric acid to the amount of said polymer being within the limits of 65:35 and 35:65.

14. A water-insensitive yarn having a size coating comprising a partially saponified polyvinyl acetate, boric acid and a polymer of the class which consists of modified polymers of dioxolane and alkyl substituted dioxolanes, said polymer being a water-soluble waxy solid, having a molecular weight within the range of 500 to 1500, and modified by a member of the class which consists of carboxylic acids and esters thereof, the ratio of the total amount of said polyvinyl acetate and boric acid to the amount of said polymer being within the limits of 65:35 and 35:65.

15. A yarn formed of a synthetic linear polycarbonamide wherein the average number of carbons in the segments of the chain separating the amide groups is at least two and having a size coating comprising a water-sensitive hydroxylated polyvinyl resin, boric acid and a polymer of the class which consists of modified polymers of dioxolane and alkyl substituted dioxolanes, said polymer being a water-soluble waxy solid and having a molecular weight within the range of 500 to 1500 and modified by a member of the class which consists of carboxylic acids and esters thereof, the ratio of the total amount of said polyvinyl resin and boric acid to the amount of said polymer being within the limits of 65:35 and 35:65, and the

boric acid being present in an amount of from 5% to 25% based on the weight of the hydroxylated polyvinyl resin.

16. A yarn formed of a synthetic linear polycarbonamide wherein the average number of carbons in the segments of the chain separating the amide groups is at least two and having a size coating comprising a partially saponified polyvinyl acetate, boric acid and a polymer of the class which consists of modified polymers of dioxolane and alkyl substituted dioxolanes, said polymer being a water-soluble waxy solid, having a molecular weight within the range of 500 to 1500, and modified by a member of the class which consists of carboxylic acids and esters thereof, the ratio of the total amount of said polyvinyl acetate and boric acid to the amount of said polymer being within the limits of 65:35 and 35:65.

17. A yarn formed of a synthetic linear polycarbonamide wherein the average number of carbons in the segments of the chain separating the amide groups is at least two and having a size coating comprising a partially saponified polyvinyl acetate, boric acid and a polymer of the class which consists of modified polymers of dioxolane and alkyl substituted dioxolanes, said polymer being a water-soluble waxy solid, having a molecular weight within the range of 500 to 1500, and modified by a member of the class which consists of carboxylic acids and esters thereof, the ratio of the total amount of said polyvinyl acetate and boric acid to the amount of said polymer being within the limits of 65:35 and 35:65, and the boric acid being present in an amount of from

5% to 25% based on the weight of the polyvinyl acetate.

18. A yarn formed of a synthetic linear polycarbonamide wherein the average number of carbons in the segments of the chain separating the amide groups is at least two and having a size coating comprising a partially saponified polyvinyl acetate, boric acid and polydioxolane sebacate, the ratio of the total amount of said polyvinyl acetate and boric acid to the amount of said polydioxolane sebacate being within the limits of 65:35 and 35:65.

19. A yarn formed of a synthetic linear polycarbonamide wherein the average number of carbons in the segments of the chain separating the amide groups is at least two and having a size coating comprising a partially saponified polyvinyl acetate, boric acid and polydioxolane adipate, the ratio of the total amount of said polyvinyl acetate and boric acid to the amount of said polydioxolane adipate being within the limits of 65:35 and 35:65.

20. A yarn formed of a synthetic linear polycarbonamide wherein the average number of carbons in the segments of the chain separating the amide groups is at least two and having a size coating comprising a partially saponified polyvinyl acetate, boric acid and polydioxolane stearate, the ratio of the total amount of said polyvinyl acetate and boric acid to the amount of said polydioxolane stearate being within the limits of 65:35 and 35:65.

HARRY R. DITTMAR.